

# United States Patent Office

3,265,497

Patented August 9, 1966

1

3,265,497

## ELECTROPHOTOGRAPHIC MATERIAL

Horst Kosche, Duren, Rhineland, North Rhine-Westphalia, Germany, assignor to Firma Renker-Belpa G.m.b.H., Lendersdorf-Krauthausen, near Duren, Rhineland, Germany

No Drawing. Filed Apr. 23, 1962, Ser. No. 191,389  
Claims priority, application Germany, Apr. 29, 1961,

R 30,222

11 Claims. (Cl. 96—1.1)

By the term "electrophotography" are understood reproducing or recording processes in which latent electric charge patterns are developed. Conventionally, the electrophotographic material is in the form of a backing to which a photoconductive layer is applied, with or without the interposition of auxiliary layers and/or electrical barrier layers. The photoconductive layer is very photosensitive when charged electrically. If the charged electrophotographic material is exposed, a latent charge pattern is produced, the electrostatic charge being reduced or eliminated at those parts of the electrophotographic layer which have been exposed to the light or radiation but remaining at non-irradiated parts. The latent charge pattern can be developed by means of appropriate liquid or solid triboelectric developer systems.

The photosensitive photoconductive layer of this electrophotographic material is produced by using special substances which can be called photoconductors without any limitation as to the mechanism of their action. A very wide variety of organic and inorganic substances have been proposed as photoconductors for use in electrophotographic layers, such as oxides, sulphides, selenides or arsenides of zinc, lead, cadmium, antimony, tin, and arsenic sulphide, lead chloride, sulphur, anthracene and pyrazoline derivatives, according to Federal German patent specification 1,060,714, 1,3,4-triazole substances according to Federal German patent specification 1,060,260, azomethines according to Federal German patent specification 1,060,712, and poly-nuclear aromatic compounds according to Federal German patent specification 1,060,259. To produce the electrophotographic layer, these photoconductors are used in combination with a bonding agent of an insulating nature with or without an addition of substances which increase the water-repellant character of the whole. However, nothing so far can be gathered from the large number of such different substances which enables accurate statements to be made about the construction of such organic compounds as can be used as photoconductors.

It has surprisingly been found that very useful and surprisingly effective electrophotographic materials can be prepared if photoconductors in accordance with the general Formulae I, II and III are used:



where Ar and Ar<sub>1</sub> denote an aromatic or heterocyclic cyclic system having free electron pairs, such as, for instance, benzene, naphthalene, diphenyl, anthracene, anthraquinone, polynuclear organic cyclic systems such as chrysene, perylene, fluorene or the like or pyridine, thiophene, coumarone, acridine, quinoline, imidazole, pyrazole, indole, pyrimidine or the like; X denotes one or more

2

substituents adhering to the aromatic or heterocyclic ring system, such as —H, —halogen,



—NH—Ac, —NAc<sub>2</sub>, —O—Ac, —cyclic secondary amine such as morpholine, piperidine, —NH—R, —NH<sub>2</sub>, —OH—SH, —COOH, —COOR, CONH<sub>2</sub>, —CONHR, CONR<sub>2</sub>, ==O, ==S, ==SO, —SO<sub>2</sub>NH<sub>2</sub>, —SO<sub>2</sub>NHR, —SO<sub>2</sub>NR<sub>2</sub>, —R, —OR, —NO<sub>2</sub>, —NO, —CH—CH—CN; R denotes an aliphatic or aromatic or cycloaliphatic saturated or unsaturated radical, such as, for instance methyl, ethyl,  $\beta$ -oxyethyl, propyl, butyl, cyclohexyl, phenyl, diphenyl, allyl, ethylene which can comprise other substituents, such as —OH, —NH<sub>2</sub>, —OR, —NHR, —Cl, —CN, —SH, —COOH, —COOR or the like; Y denotes an oxygen or sulphur atom; Ac denotes an acid radical, preferably that of an organic carboxylic acid, such as formyl, acetyl, or benzoyl, it being possible for di- or poly-carboxylic acids, such as malonic acid, oxalic acid, maleic acid, succinic acid, adipic acid, phthalic acid or terephthalic acid, trimesic acid, tartaric acid, citric acid or their substitution products to be reacted repeatedly with substances having the general Formulae I—III; n<sub>1</sub> denotes a whole number from 2 to 3; and n<sub>2</sub> denotes a whole number from 1 to 3.

The Ar and Ar<sub>1</sub> grouping and the X substituents can be so disposed that symmetrical and asymmetrical compounds are produced which can comprise the X substituents in different ways and a number of times. Ar and Ar<sub>1</sub> may or may not belong to the same cyclic system. Symmetric and asymmetric compounds are suitable as electrophotographically active substances. The introduction of the



groups or cyclic secondary amine as X substituent in at least one cyclic system is particularly valuable. A simple symmetrical type which is highly active is the tetramethyl-4,4'-diaminobenzophenone known as "Michler's ketone."

The compounds according to the formulae given herein represent ketones or thioketones and can be prepared by a wide variety of known methods. Conveniently, to prepare ketones having the general Formula I and comprising a dialkyl amino group on the cyclic system, the analides of an aromatic or heterocyclic carboxylic acid, which may or may not be correspondingly substituted, are used as starting material and are reacted, using condensation agents, more particularly phosphoroxychloride, with tertiary aromatic amines having a free p-position and the reaction product is broken down with acids to the ketone. Appropriate tertiary amines are, for instance, dimethyl aniline, diethylaniline, ethyl-( $\beta$ -oxyethyl)-aniline, phenylmorpholine, ethyl-( $\beta$ -acet-oxyethyl)-aniline,  $\alpha$ -dimethylaminonaphthaline, phenylpiperidine - N' - acetate, N-methyl-diphenylamine and so on.

Substances having the general Formula II are, of course, prepared by condensation of aromatic or heterocyclic methyl ketones with unsaturated aldehydes. Substances having formula III are prepared either—in the case of symmetrical compounds—by condensation of 2 mol of the aldehyde with 1 mol of acetone, with the action of alkaline or acid condensation agents, or—in the case of asymmetrical compounds—by condensation of styryl-methyl-ketones and aldehydes. When X substituents are used which can react with the aldehyde, such substituents

are, with advantage, masked before the reaction is performed.

Of particular value in the preparation of self-adhesive photoconductors are those compounds having the general Formulae I-III which contain one or more substituents reactable with epoxy and/or isocyanate groups, possibly at different reaction rates, and which contain reactable hydrogen one or more times in the molecule, possibly besides other substituents or sticking to the R substituent, as, for instance, in the  $-\text{OH}$ ,  $-\text{SH}$ ,  $-\text{NH}_2$ ,  $-\text{NHR}$ ,  $-\text{COOH}$ ,  $-\text{CONH}_2$ ,  $-\text{CONHR}$ ,  $-\text{SO}_2\text{NH}_2$ ,  $-\text{SO}_2-\text{NHR}$ ,  $-\text{NH}-\text{CO}-\text{NH}_2$ ,  $=\text{CH}_2$  or  $=\text{O}$ ,  $=\text{S}$  and  $=\text{NO}$ . These photoconductors which correspond to the general Formulae I-III and which are reactable with epoxies or isocyanates are reacted, to produce self-adhesive photoconductors, with isocyanate-and/or epoxy-group-containing compounds, with or without an addition of other participants in the condensation which are not photoconductors, to provide electrophotographically active resin-like substances with marked adhesion on metals, ceramic products, papers, plastics, glasses and fabric materials. The following compounds were prepared in accordance with the general Formulae I-III, the number denoting the structural formula:

- (1) Tetramethyl-4,4'-diamino-benzophenone
- (2) Tetramethyl-4,4'-diaminothiobenzophenone
- (3)  $\text{N}''\text{,N}'''$ -tetramethyl-di- $\alpha$ '-amino-di- $\beta$ -pyridyl-thioketone
- (4) 4,4'-dimethyl-diamino-3,3'-dimethylthiobenzophenone
- (5) dimethyl-4-amino-thiobenzophenone
- (6) 4,4'-dimethoxy-thiobenzophenone
- (7) 4-dimethylamino-4'-nitro-benzophenone
- (8) 4-dimethylamino-4'-amino-benzophenone
- (9) 4,4'-dimethoxy-benzophenone
- (10) 4-dimethylamino-4'-chlorobenzophenone
- (11) Phenyl- $\alpha$ -thienyl-ketone
- (12) 4-dimethylamino- $\alpha$ -naphthyl-4'-nitrophenyl-ketone
- (13) 4-dimethylamino- $\alpha$ -naphthyl-4'-aminophenyl-ketone
- (14) 4-N-ethyl-( $\beta$ -oxyethyl)-amino-benzophenone
- (15) di-(quinolyl)-(6)-ketone
- (16) 4-dimethylamino-4'-methylanilino-benzophenone
- (17) 3-nitro-4,4'-bis-dimethylamino-benzophenone
- (18) 3-amino-4,4'-bis-dimethylamino-benzophenone
- (19) 4-dimethylamino-3'-nitro-benzophenone
- (20) 2-oxy-4-diethylamino-benzophenone-carboxylic acid-(2')
- (21) 2-oxy-4-diethylamino-benzophenone-carboxylic acid-(2')-methyl-ester
- (22) 4-dimethylaminophenyl-3'-oxynaphthyl-2'-ketone
- (23) 4-[methyl-( $\beta$ -hydroxyethyl)-amino]-cinnamal-4'-diphenyl-acetophenone
- (24) 4-[methyl-( $\beta$ -hydroxyethyl)-amino]-cinnamal-3'-nitro-acetophenone
- (25) 4-dimethylamino-cinnamal-3'-amino-acetophenone
- (26) 4-[methyl-( $\beta$ -hydroxyethyl)-amino]-cinnamal-2'-hydroxy-4'-dimethylamino-acetophenone
- (27) 4,4'-bis-dimethylaminodibenzylidene-acetone
- (28) 2,2'-bis-( $\beta$ -methylamino-ethyl)-benzal
- (29) Phenyl-(1-amino-anthraquinolyl)-(2)-ketone
- (30) 9-hydroxy-4-benzoyl fluorene
- (31)  $\alpha$ -anisylidene- $\alpha$ -(3-nitro-cinnamylidene)-acetone
- (32) (4-dimethylamino-phenyl)-4'-methylamino-naphthyl-(1')-ketone
- (33)  $\alpha$ -(4-[methyl-( $\beta$ -hydroxyethyl)-amino]-cinnamylidene)- $\alpha$ '-(4'-nitro-toluylene)-acetone
- (34) 3,5-dinitro-4'-diethylamino-benzophenone
- (35) 4-[methyl-( $\beta$ -hydroxyethyl)-amino]-cinnamal-acetyl-acenaphthene
- (36) 2,2'-carboxy-benzoyl-7-dimethylamino-fluorenone

- (37) 2-[2'-(carboxy-mono-glycol ester)-benzoyl]-7-diethyl-amino-fluorenone
- (38) x,x'-[bis-dimethylamino-]bis-p-diphenyl-ketone
- (39) 1,1'-carbonyl-di-indazole
- (40) 1-(4'-nitrobenzoyl)-indazole
- (41) 1-(4'-dimethylaminobenzoyl)-6-nitro-indazole
- (42) 1-(4'-dimethylaminobenzoyl)-3-(4''-dimethyl-amino-phenyl)-indazole
- (43) 1-(4'-diethylaminobenzoyl)-6-nitro-benzimidazole
- (44) 1-(2'-carboxy-phenyl)-benzimidazole
- (45) 2-(4''-diethylaminobenzoyl)-3-hydroxy-diphenyl
- (46) 2-(4''-diethylaminobenzoyl)-3-hydroxy-4'-diethylamino-diphenyl.

15 The photoconductors according to the invention differ in their spectral sensitivity. For instance, Compound 22 is sensitive only to the spectrum of incandescent light, while with others it is convenient to add sensitizers to adapt the photoconductive layer to the spectral range 20 of desired light sources. As a rule, this increases the photosensitivity. As sensitizers there can be used, for instance, the sensitizers conventional in silver halide photography. They can be used in a proportion of from 0.2 to 3% referred to the compounds having the general Formulae I-III. For instance, the sensitizers disclosed by French patent specification 1,288,292 are suitable.

25 To produce the photoconductive layers, the photoconductors, which correspond to the general Formulae I-III and which comprise X substituents and which can react with epoxies and/or isocyanates, more particularly such photoconductors as have active hydrogen atoms, are, after reaction with isocyanates and/or epoxies, reacted to form self-adhesive photoconductors. Highly photosensitive 30 photoconductive layers can be prepared from these self-adhesive photoconductors without the use of bonding agents. Such layers do not have any of the grain structure of the photoconductor. Photoconductive layers can also be prepared by compounds corresponding to the general Formulae I-III or the self-adhesive photoconductors prepared from such compounds being used in a mixture or in solutions with bonding agents. Other photoconductors, such as zinc oxide, can be added. The bonding agents can be natural and synthetic resins, with or without 35 an addition of plasticisers. A number of bonding agents are disclosed in French patent specification 1,288,392. The bonding agents can either be dissolved in solvents or used as aqueous dispersions, depending upon their properties, in combination with one or more electrophotographically active compounds of the general Formulae I-III, with or without an addition of sensitising dyes, to produce the photoconductive layer. Bonding agents which in combination with solvents dissolve the 40 photoconductors are convenient.

45 55 The proportion of electrophotographically active substances corresponding to Formulae I-III to bonding agents can vary within wide limits, and the charging time and photosensitivity can be varied by such proportion being varied; the same can also be used to control the ability 60 to store latent electrostatic charge patterns for a prolonged time.

55 The photosensitivity of the photoconductive layer also depends upon its thickness. A thickness of from 0.002 to 0.1 mm., more particularly from 0.004 to 0.008 mm., 65 is very satisfactory. Above a critical thickness of the layer or emulsion, the image is reversed from positive to negative. This effect is technically useful for the preparation of reversal material.

65 To produce electrophotographic material, the preparation which forms the photoconductive layer is applied to an appropriate backing material by some form of conventional treatment, such as lacquering, centrifuging, spraying, electrostatic spraying, printing, coating with 70 coating rollers and scraping off with doctor devices, dipping, reeling, pressing with grooved dyes, or in the form 75

of a foil, with subsequent lining, or by means of an extruder. If required, the preparation can be embedded in the form of a thin continuous layer in the backing material.

A very wide variety of substances, preferably in some sort of flat form, can be used as backing material for electrophotographic materials. Backing materials which are not so conductive electrically as is the photoconductive layer are very useful. In particular, metal plates or foils, including those which have undergone changes in surface composition by electrical or chemical treatment, papers, fabric fleeces, electrically conductive plastics and foils, electrically conductive ceramic products and so on have proved satisfactory as backing materials. Papers or foils which have been vapour coated with metals, supports which have been connected to metal foils, papers or fibre fleeces which have been rendered conductive by an addition of electrolytes or of moisture stabilisers, or such supports as have electron-conductive substances, such as powdered metal, carbon black or graphite embedded in them, are particularly suitable. Also suitable are plastics containing metals or metal compounds, carbon or a large proportion of electrolyte. Non-conductive backings can be provided with a conductive layer of lacquer on their surface. A very wide variety of combinations is therefore possible.

Uniformity in the thickness of the photoconductive emulsion has a very great effect on the quality of the finished image. Advantageously, therefore, backings having a non-uniform surface are provided with an auxiliary layer which forms a smooth and closed surface. This auxiliary or intermediate layer can be so devised as, if required, to increase and equalise the conductivity of the backing material and to improve the adhesion and anchorage of the electrophotographic layer on the backing. Preferably, the substances used for the intermediate layer are substances which are dissolved or changed little, if at all, by the preparation which leads to the electrophotographic layer. Organic water-soluble colloids have proved very useful for these purposes. Such substances are, for instance, cellulose ethers, such as methyl celluloses and cellulose glycol acids, including those which have been partly reacted with ethylene oxide or propylene oxide, starch ethers, casein, polyuronides, the salts or amides thereof, ethylene or propylene oxide reaction products, natural colloids, such as Irish moss, starches, including broken-down starches, gelatin, lichenin, agar-agar, tragacanth, hydrate celluloses, and synthetic resins, such as polyvinyl alcohol, polymethacrylic acid and its acetals, methyl hydantoin resins, maleinate-polyacrylic acid resins or others which contain free carboxyl groups and are water-soluble in their salt form. A further increase in the electrical conductivity of the emulsions can be provided by an addition of soots, metal powders or electrolytes and moisture stabilisers, such as sorbitol, polyglycol ethers, broken-down starches or hygroscopic metal salts.

Photoconductive emulsions prepared by the process according to the invention are also of use in the preparation of printing plates such as are used, for instance, for offset printing. For this purpose, the photoconductive layer is produced from compounds having the general Formulae I-III, preferably in their form as self-adhesive photoconductors, possibly in combination with bonding agents or other photoconductors, such as zinc oxide. Particularly good electrophotographic emulsions for printing can be prepared from the self-adhesive photoconductor type reaction products of those compounds according to Formulae I-III comprising substituents which can react with isocyanates and/or epoxies to form resin-like substances. The solubility of the electrophotographic emulsions can be varied within wide limits by using appropriate compounds which contain isocyanate and/or epoxy groups and by reaction with other substances which are not photoconductors.

To this end, pretreated papers, plastic foils or fabrics,

or possibly a colloidal or resin emulsion in the form of a combination or selection of gum arabic, caseinates, polyuronide salts, more particularly their zinc salts, dextrines, starches, starch ethers, polyvinyl alcohols including those containing acetate or acetal groups, agar-agar, zinc salts of resin or fatty acids, polyacrylates or polymethacrylates, amides of polyacrylic acids, cellulose ethers and gelatin, are applied to a backing which has been pretreated to make it suitable for printing purposes, such as metal foils which have been galvanically treated by oxidation, for instance, by eloxation or by aloidinisation or which have a very finely roughened surface. The preparation forming the photoconductive layer is applied by appropriate applicators, preferably mechanically, to this backing material which has been pretreated to make it stick and/or to make it take up water or which has been provided with hydrophilic intermediate layers, whereafter the photoconductive layer or emulsion is dried. The electrophotographic emulsion should be such that the self-adhesive photoconductors, using compounds having the general Formulae I-III, or the electrophotographically active substances having the general Formulae I-III and also the bonding agent are soluble in conventional solvents or in water, whereas the toner used to produce the image must not be attacked by the same solvents.

Conveniently, the bonding agent is hydrophilic, so that the non-de-emulsified developed printing plate can be used for printing immediately after wetting.

The process for preparing printing plates can also be used, of course, to prepare etched engravings, for instance, in the preparation of impression rollers or stereo blocks, and in the preparation of printed circuits. The toner, in a form resistant to acid and in a fused-in state, then serves as masking agent, while the photoconductive layer not required for image production is removed before etching by conventional etching agents, preferably from the metallic support.

#### Example 1

20 g. of phenyl- $\alpha$ -thienyl-ketone in accordance with Formula 11 are dissolved with slight heating in 100 cc. of ethyl acetate, and there is added to this mixture a solution of 40 g. of a copolymer of vinyl chloride and vinyl acetate (commercial product known as Vinylite VAGH) in 30 cc. of ethyl acetate and 50 cc. of butyl acetate. To produce the photoconductive emulsion, the solution just described is applied in a centrifuge to an electrochemically polished and eloxated aluminium foil. The colourless electrophotographic plate is charged to  $-7$  kv. under a corona discharge type electrode arrangement, the positive electrode being formed as a baseplate on which the electrophotographic material is supported. The negative electrode is in the form of thin tungsten wires which are from about 0.02 to 0.1 mm. thick and which are at a distance of from 10 to 15 mm. from the electrophotographic plate and at a distance of 15 mm. from one another. This arrangement is conventionally used to charge the electrophotographic material. If the tungsten wires are made positive in the baseplate negative, the electrophotographic plate is charged positively. The charged electrophotographic material is exposed below an original with a high-pressure mercury vapour lamp for 20 seconds, then developed by means of a triboelectric system comprising a toner and glass balls, the toner being made of plastics, colouring agents and/or soots. If the toner known commercially as the Graph-O-Fax-Toner No. 39/50, of the P. A. Hunt Company, and glass balls are used, a positive original gives a positive image which can be fixed by being heated to  $120^{\circ}$  C. or by the action of solvent vapours.

The electrophotographic material can be used for image transfer in an electric field to other, preferably sheet-like substances, such as paper, plastics foil or the like. Adequate sensitivity for working with incandescent light can be produced by an addition of from 0.1 to 1% of sensi-

tising colouring agents to the coating solution, referred to the photoconductor, such as Rhodamin B (Schultz-Farbstofftabellen, Leipzig 1931, No. 864) or brilliant green (Schultz-Farbstofftabellen, Leipzig 1931, No. 760).

*Example 2*

2 g. of 4-dimethylamino-4'-aminobenzophenone in accordance with Formula 8 are dissolved in 10 cc. of methyl ethyl ketone and 10 cc. of dimethyl formamide and added to a solution consisting of 4 g. of a colophonymaleic acid resin, for instance, the commercial product known as Alresat 313c, and 1 g. of ethyl cellulose, for instance, the commercial product known as ethyl cellulose N200, dissolved in 40 cc. of aceto-ethyl. A thin coating of this solution is applied to a pretreated paper support which cannot be penetrated by the emulsion solution and which has been made ionically conductive by impregnation. After evaporation of the solvents a slightly yellowish electrophotographic material is yielded on which images can be produced directly. To this end, the material is charged up to -8 kv. as described in Example 1, placed below a positive original and exposed to ultra-violet fluorescent tubes. When the material is developed with a soot-stained resin powder and glass balls or iron filings in association with a magnet, a high-contrast positive image is produced at the unexposed places and is fixed by slight heating and/or solvent vapours. An addition of Rhodamin B and Pinacyanol blue is useful to increase the sensitivity to incandescent light.

*Example 3*

5 g. of 4-dimethylamino-4'-nitro-benzophenone in accordance with Formula 7, and 11 g. of a ketone or ketone-aldehyde resin, for instance, the synthetic resin commercially known as AP, are dissolved in 100 cc. of methyl ethyl ketone and 25 cc. of dimethyl formamide with heating and used to coat an aluminium plate in a centrifuge. After removal of the solvents, the applied layer sticks tightly to the support. This electrophotographic material is used to produce an image in the manner described in Example 1. The produced and still unfixed and, for instance, positively charged powder image is covered with a sheet of paper, with a waxed paper or with resin-impregnated paper or with a plastics foil and is so introduced into an electric field produced by a voltage of from 2 to 6 kv. at a spacing of 20 mm. that the negative electrode is associated with the back of the sheet of paper. The, for instance, positively charged toner is therefore transferred to the sheet material in laterally inverted form and can be fixed by heating and/or solvent vapours. Contact copies on a transparent material can be used as intermediate originals for other photocopies, for instance, photo-prints, for projection purposes and so on.

*Example 4*

31 g. of 2-oxy-4-diethylamino-benzophenone-carboxylic acid (2) according to Formula 20, and 0.3 g. of Rhodamin B, are dissolved with heating in 100 cc. of cyclohexanone. There are added to the cooled solution 47 g. of a reaction product which contains three free isocyanate groups in the molecule and which has been prepared from 1 mol of 1-trimethylol propane and 3 mol of toluylene-2,4-diisocyanate and/or toluylene-2,6-diisocyanate (commercial product known under the trade mark of Desmodur L), 75% by weight in an ethyl acetate, dissolved in 100 cc. of cyclohexanone. The mixture is condensed at 151° C. with reflux boiling for 20 minutes, the viscosity increasing considerably. The condensation gives the reaction product dissolved in cyclohexanone limited compatibility with acetone. If the reaction product is mixed with acetone in the proportion of 10:1, the self-adhesive photoconductor separates out. The reaction should be so controlled that no three-dimensional cross-linking occurs. 25 g. of the reaction solution are mixed with 25 cc. of methyl ethyl ketone and 35 cc. of dioxane and, after filtration, used to

prepare the electrophotographic layer, an electrochemically polished aluminium foil being so coated in a centrifuge that a layer thickness of about 0.006 mm. dry is produced. The coated plate is dried by ultra-red radiation on the centrifuge, then baked at 130° C. for 5 minutes. A lustrous very strong electrophotographic layer which sticks fast mechanically to the backing is produced. It is charged electrostatically at -7 kv. for 3 seconds, exposed below an original with ultra-violet fluorescent tubes for 1 second, then developed using glass balls and a direct toner. A high-contrast electrophotographic image is produced.

Another method of producing an image is for the electrophotographic plate just described to be exposed when charged through a microfilm, and for a time of 25 seconds, in an enlarger having a 150 watt cine-projection lamp, with an aperture ratio of 1:5.6 with a distance of 30 cm. between the lens and the plate. A high-contrast electrophotographic image is yielded after development.

The still unfixed electrophotographic recordings can be transferred in an electric field to other substances, preferably in sheet form, as described in Example 1.

*Example 5*

145 g. of 4-N-ethyl-( $\beta$ -oxyethyl)-aminobenzophenone according to Formula 14 are reacted with 300 g. of ethylene glycol diglycidic ether at 170° C. in a nitrogen atmosphere for 30 minutes, whereafter 190 g. of ethylene glycol diglycidic ether boiling at from 142-167° C./3 torr. are distilled off in a vacuum produced by an oil pump. The resin which remains as residue is dissolved hot in 500 cc. of cyclohexanone and to this solution there are added 200 g. of a modified isocyanate (the commercial product called Desmodur L) in a proportion of 75% by weight in ethyl acetate, and condensation is effected at 100° C. (usually for 5 minutes) until the solution is still compatible with methyl ethyl ketone and no gelatinisation occurs. 100 cc. of the cooled reaction solution thus prepared are diluted with 200 cc. of methyl ethyl ketone. This solution is applied in a uniform thickness of 0.008 mm. to a highly lustrous aluminium foil. The photoconductive layer formed is dried in an air stream first at 120° C. and then for a short time at 140° C. The electrophotographic material formed, when charged as set forth in Example 1 to -7 kv. and exposed under a positive original with a high-pressure mercury vapour lamp or a pulse discharge tube, yields upon development a high-contrast positive reproduction which can also be used for image transfer.

*Example 6*

77 g. of 4-dimethylamino-4'-amino-benzophenone according to Formula 8 are dissolved in 300 cc. of cyclohexanone, 88 g. of a modified triisocyanate (commercial product called Desmodur L) in a proportion of 75% by weight in ethyl acetate, dissolved in 200 cc. of cyclohexanone, are added and condensing with reflux boiling is effected at from 145 to 152° C. for 30 minutes. To prepare the electrophotographic material, a plastics-impregnated smooth-surfaced glass fibre fleece which has had aluminium vapour coated onto its smooth side is used as backing material. A solution consisting of 50 cc. of the reaction product just described diluted with 100 cc. of methyl ethyl ketone and 0.3 g. of erythrosine (corresponding to the Schultz-Farbstofftabellen 1931, No. 886) and 0.2 g. of brilliant green (corresponding to the Schultz-Farbstofftabellen 1931, No. 760) are applied to the backing material in a centrifuge, dried with ultra-red radiation and baked at 120° C. A flexible firmly adhering electrophotographic layer having considerable abrasion resistance is produced and can be used as set forth in Example 1 in the preparation of electrophotographic reproductions. The electrophotographic material is very sensitive to incandescent light.

*Example 7*

105 g. of 4-[methyl-( $\beta$ -hydroxyethyl)-amino]-cinnam-

al - 2' - hydroxy - 4' - dimethylamino-acetophenone corresponding to Formula 26 are dissolved in 300 cc. of cyclohexanone, and 88 g. of a modified triisocyanate (commercial product called Desmodur L), in a proportion of 75% by weight in ethyl acetate, are added and reacted at 150° C. for 20 minutes. 100 cc. of the reaction solution are mixed with 50 cc. of methyl ethyl ketone and with 50 cc. of ethyl amyl ketone and painted onto an aluminium foil which is dried in an air stream at 120° C. The electrophotographic material is charged up to -6 kv. and exposed under a positive original with a high-pressure mercury vapour lamp or an arc lamp or ultra-violet fluorescent tubes. Using a toner having a particle size of from 10 to 50  $\mu$  and glass balls, a high-contrast positive image of the original is produced which can be fixed by heating and/or solvent vapours.

To transfer the image to other flat materials, such as papers or plastics foils, the unfixed image on the electrophotographic plate is brought into intimate contact with sheet material and so introduced into an electric field that, for instance, the negative electrode is disposed behind the sheet material. If the electric field is strong enough, for instance, of 6 kv./20 mm., printing is effected by the field strength alone. By intermediate changes of a field of differing field strength and direction, varying quantities of toner can be transferred and a number of copies can be prepared from one image on the electrophotographic plate. The transfer image is fixed like the electrophotographic plate.

#### Example 8

28 g. of 4-dimethylamino-cinnamal-3'-aminoacetophenone in accordance with Formula 25 are prepared fresh, introduced into a solution consisting of 50 g. of an epoxy resin of the type formed by diphenol propane which has been reacted with epichlorohydrin and which has been partly condensed with itself with molecule enlargement (commercial product known as Epikote 1001 Shell), in 250 cc. of ethyl amyl ketone, and dissolved with heating and agitation. The solution is kept at about 100° C. with reflux boiling for 20 minutes, its viscosity increasing considerably. 100 cc. of reaction product are diluted with 50 cc. of methyl isobutyl ketone and 50 cc. of methyl ethyl ketone, and to this are added, to produce a non-sticky surface, 5 g. of a modified triisocyanate (commercial product called Desmodur L), 75% by weight in ethylacetate, and 0.2 g. of Rhodamin B as per Schultz-Farbstofftabellen 1931, vol. 1, No. 864 and 0.1 g. of pinacyanol as per Schultz Farbstofftabellen 1931, vol. 1, No. 924, then used immediately to produce the electrophotographic layer.

The backing material is a copper foil which has a smooth front but a spongy back and which is connected on the back to a resilient high-melting plastic or to rubber. The dissolved self-adhesive photoconductor is applied to the front of this backing material and dried in an air stream at 100° C. to remove the solvents, whereafter the front is given a brief radiant heat treatment at 120° C.

#### Example 9

50 g. of 4-dimethylaminophenyl-3' - oxynaphthyl - 2'-ketone in accordance with Formula 22 are dissolved in 200 cc. of cyclohexanone, 104 g. of the isocyanate ingredient to be described hereinafter, 52% by weight in cyclohexanone, are added and condensing is effected at 135° C. for 10 minutes. 50 cc. of the reaction product are diluted with 50 cc. of methyl ethyl ketone and with 50 cc. of ethyl amyl ketone and filtered. The isocyanate ingredient is prepared by reaction of 32 g. of 2-ethyl-2-butyl-propanediol-1,3 with 70 g. of toluylene-2,4-(or 2,6) diisocyanate in 300 cc. of cyclohexanone at 148° C. for 3 hours. Small traces of toluylene-2,4-(or 2,6) diisocyanate are removed from the solvent-free reaction product by molecular distillation. The reaction product contains about 17% by weight of free isocyanate groups. This

solution of self-adhesive photoconductor is applied by applicator comprising dispensing rollers onto an aluminium-vapour-coated cellulose paper having a density of 80 g./m.<sup>2</sup>, dried in a warm air stream, then given brief afterheating at 120° C.

Because of its green colour, the self-adhesive photoconductor is very photosensitive. When charged up in a coronary discharge arrangement to -7 kv., then exposed below a positive original with ultra-violet cold light tubes for 3 seconds, the substance, after development with glass powder and a direct toner, provides a high-contrast positive image which is fixed by heating or by solvent vapours.

Another generally applicable development method is the use of so-called liquid developers comprising a dispersion of dye particles with an addition of soluble or dispersed plastics in a liquid medium. With this method, similarly to the development by means of powdery developers of electrophotographic layers or emulsions prepared from self-adhesive photoconductors, development can be effected if the liquid phase of the developer is such that the electrophotographic emulsion is not dissolved. Preferably, the photoconductive emulsions prepared from self-adhesive photoconductors are of the kind which still contain reactable isocyanate and/or epoxy groups and are given three-dimensional cross-linking during the production of the electrophotographic emulsion. To this end, small quantities of polyamines, polycarboxylic acids or polyalcohols are added to the preparation which will subsequently lead to the electrophotographic layer, and cross-linking is effected during drying by the use of heat.

#### Example 10

35 15 g. of a chlorinated diphenyl resin, for instance, the commercial product called Clophenharz W, and 3 g. of a broken-down natural rubber, for instance, the commercial product known as Cyclosit, are heated to 150° C. to produce a homogeneous melt. 5 g. of tetramethyl-4,4'-diaminobenzophenone in accordance with formula 1 are dissolved in the melt, whereafter the same is used, at a temperature of from 140 to 150° C., to coat heat-stable backing materials for electrophotography, for instance, by the melt being applied to aluminium sheet which has been heated to 140° C.

45 Emulsion thicknesses of from 0.005 to 0.01 mm. are very useful to provide short exposure times and a substantially colourless emulsion. The electrophotographic material is charged up to -7 kv. and exposed below a positive original with ultra-violet fluorescent tubes for 15 seconds. After development as set forth in Example 1, a high-contrast positive electrophotographic image results which is fixed by heating or by solvent vapours or which can be used for transfer to other materials in an electric field. High sensitivity to incandescent light can be provided by an addition of 0.2 g. of Rose bengale (Schultz-Farbstofftabellen 1931, No. 889) 0.05 g. of Pinavflavol (Schultz-Farbstofftabellen 1931, No. 925) and 0.05 g. of Pinacyanol (Schultz-Farbstofftabellen 1931, No. 924).

55 As an alternative method of application, the electrophotographic layer is applied from the melt to the backing material by means of pressing tools which ensure a thin and uniform thickness of the emulsion. The material is ready for use immediately after cooling.

#### Example 11

65 15 g. of a hydrated colophony ester resin, for instance, the commercial product known as Staybelite-Ester 10, and 5 g. of ethylcellulose N200 are dissolved in 75 cc. of ethyl acetate, and 10 g. of 4-dimethylaminophenyl-3'-oxynaphthyl-2'-ketone in accordance with Formula 22, dissolved in 20 cc. of methyl ethyl ketone, are added. To use this solution to coat backing materials on the centrifuge, 1 part by volume is diluted with 1 part by volume of methyl ethyl ketone and with 2 parts by volume of cyclohexanone.

A 60 g./m.<sup>2</sup> cellulose paper is coated with a preparation to inhibit penetration of the electrophotographic layer and with a conductivity-promoting protective layer. The latter layer is prepared, for instance, by application of a solution consisting of:

3 g. of a film-forming methyl cellulose,  
5 g. of ammonium chloride,  
2 g. of zinc chloride,  
5 g. of sorbitol, and  
1 g. of boric acid dissolved in 100 g. of water,

and subsequent drying in an air stream at 100° C. The preparation leading to the photoconductive layer is applied to the backing material which has been thus prepared, and is dried in a stream of warm air at 120° C. The electrophotographic material can be used for image production as set forth in Example 1. When the material is charged negatively, placed under a positive original and exposed with a high-pressure mercury vapour lamp and developed, a positive image is provided.

The preparation just described for the production of the electrophotographic emulsion can also be used in the preparation of printing forms. To this end, it is applied to a backing material which has a hydrophilic surface, for instance, in the form of a colloidal layer, or which is in the form of an electrically or chemically pretreated metal foil, and the whole is dried in a warm air stream. The electrophotographic material is ready for use after drying and can be cleaned by being washed with water and/or detergents. To prepare the printing form, for instance, the electrophotographic plate is briefly charged at -7 kv., then placed below a positive original and irradiated with short-wave light either by the direct contact method or with the interposition of a microfilm in the projection method. From a positive original, a positive image is provided after development with a toner which is insoluble in alcohol and is suitable more particularly to receive printing ink, and with glass balls. To provide a firm anchorage, the toner is melted into the photoconductive layer. By removal of the emulsion with ethanol, the electrophotographic plate is converted into a printing form, that area of the photoconductive emulsion which has not been used for the image being removed. The form, after being wiped over with 30% phosphoric acid and possibly being given a further short melting-in treatment, is inked on an offset printing press with a simultaneous supply of water and printing ink. The form gives a large run with exact reproduction of the print.

#### Example 12

87.5 g. of a modified triisocyanate, formed by reacting 3 mol of 2,4-tolylene diisocyanate and 1 mol trimethylol-propane containing three free isocyanate groups (for instance, the commercial product called Desmodur L), 75% by weight in ethylacetate, 28 g. of n-dodecanol and 57.5 g. of 4-[methyl-( $\beta$ -hydroxyethyl)-amino]-cinnamal-4'-di-phenyl-acetophenone in accordance with the Formula 23, are dissolved in 200 cc. of cyclohexanone and reacted at 140° C. to a self-adhesive photoconductor which is soluble in cyclohexanone. The reaction product is diluted with 400 cc. of ethyl amyl ketone, and 1 g. of Rhodamin 3 B (No. 867), 0.3 g. of Orthochrom T (No. 923), and 0.3 g. of naphthacyanol (No. 926) are added, the numbers which follow the sensitizers referring to the Schultz-Farbtabellen, vol. 1, 1931. To prepare the photoconductive emulsion, the solution just described is so applied mechanically to a paper-lined aluminium foil, and so dried in a warm air stream at 125° C., that the thickness of the emulsion is from 0.005-0.02 mm. A firmly adhering highly photosensitive photoconductive layer is produced.

The aluminium foil of the electrophotographic material is connected to the positive side of the charging device and charged to a negative corona of 10 kv. The material is exposed, through a film bearing a positive image, in an enlarger comprising a 250-watt incandescent lamp at an

aperture ratio of 1:4.5 and at a distance of 50 cm. between the lens and the plane of the image, for 4 seconds, then developed by means of a direct-acting triboelectric system, for instance, the commercial product known as Graph-O-Fax-Toner 39/50, and glass balls, and a high-contrast positive image of the original is provided. The powder image can be fixed by known steps, such as by being heated to 120° C.

If the photoconductive emulsion is charged with a positive corona of 10 kv., exposed through a negative original and developed with a reversal toner, for instance, the commercial product known as Xerox-Toner SC13, and glass balls, a positive image of the negative original is provided.

#### Example 13

10 g. of tetramethyl-4,4'-diaminothiobenzophenone in accordance with Formula 2, and 0.3 g. of Rhodamin 3 B, corresponding to the Schultz-Farbtabellen 1931, No. 867, are dissolved in 40 g. of a chlorinated diphenyl resin, for instance, the commercial product known as Clophen Harz W, which has been heated to 120° C. This melt is used in the preparation of electrophotographic material in the manner set forth in Example 10.

#### Example 14

30 g. of 4,4'-bis-dimethylamino-di-benzylidene acetone in accordance with Formula 27, and 87.5 g. of the reaction product prepared from 3 mol of tolylene-2,4 (or 2,6)-diisocyanate and 1 mol of trimethylolpropane (for instance, the commercial product known as Desmodur L), 75% by weight in ethyl acetate, are dissolved hot in 150 cc. of cyclohexanone and 300 cc. of ethylamyl ketone. A solution of 20 g. of hexane-diol-1,6 in 100 cc. of ethylamyl ketone is added, and this freshly prepared solution is used to coat an aluminium foil to a thickness of from 0.004 to 0.05 mm. The applied and still solvent-containing photoconductive emulsion or layer is dried in a warm air stream and after-heated at 140° C. for a further 5 minutes. A firmly adhering photoconductive layer of a deep orange-reddish colour is produced which is very sensitive to incandescent light and to long-wave ultra-violet light. The electrophotographic material is charged to -6 kv. for a short time, then exposed for 5 seconds through a microfilm in an enlarger having a 250 watt cineprojection lamp, through a lens having an aperture ratio of 1:4.5, with a distance of 30 cm. between the lens and the plane of the image. After development with a triboelectric system using a direct toner and glass powder, a high-contrast positive electrographic image of high resolution is produced. The picture thus prepared can be used for image transfer in an electric field or by pressing, for instance, on paper or plastics foils. Fixing is by heating and/or solvent vapours.

#### Example 15

2 g. of 4,4'-dimethoxy-thiobenzophenone in accordance with Formula 6, 4 g. of a ketone or aldehyde resin, for instance, the synthetic resin known commercially as 60 AP, and 1 g. of 65% collodion wool, wetted with ethanol, are dissolved in 4 cc. of ethanol, 60 cc. of acetone and 20 cc. of butyl acetate. The solution is used to coat a 0.3 mm. thick aluminium foil in a centrifuge, the coating being uniform, whereafter drying is effected in an air stream at 120° C. The electrophotographic material has a high metallic lustre and a slight blue tinge. When the material is charged to -7 kv. and exposed with a high-pressure mercury vapour lamp below a positive original, a high-contrast positive electrophotographic image of high storage capacity is produced.

It is usually possible, after removal of the powder image, recharging and exposure below a different original, to produce a second electrophotographic image on the same electrophotographic plate after repetition of the steps of the process. However, when the electrophoto-

graphic material just described is recharged to -7 kv. after removal of the first image and is exposed to the same light source but without any original, the image first produced is produced again after development. This latent electrostatic image is very difficult to destroy just by alteration of the field direction during charging but can be expunged by heating to 80° C. or by treatment with water or water vapour. This electrophotographic material is suitable for storing latent electrostatic charge patterns.

*Example 16*

10 g. of 2-oxy-4-diethylamino-benzophenone-carboxylic acid (2')-methyl ester in accordance with Formula 21, 0.2 g. of Rhodamin B (Schultz-Forbstofftabellen No. 864), and 17.5 g. of a modified isocyanate having three reactable isocyanate groups in the molecule, for instance, the commercial product known as Desmodur L, are dissolved in 45 cc. of cyclohexanone and condensed with reflux boiling for 30 minutes. The solution is cooled to room temperature, then 5.6 g. of di-(2-ethylhexyl)-amine dissolved in 20 cc. of cyclohexanone are added and the mixture is reacted at 100° C. for 10 minutes.

The photoconductive emulsion produced from this self-adhesive photoconductor is readily soluble in lower aliphatic alcohols and is very sensitive to incandescent light. It is very useful for producing electrophotographic material for use in printing forms, more particularly for offset printing. To this end, the solution of self-adhesive photoconductor, preferably in a very dilute condition, is applied to a print support and dried. As print supports there are suitable papers which have been pretreated with a colloidal emulsion, aluminium foils which have been surface-phosphated or eloxated, and aluminium foils which have been pretreated galvanically or by brushing or etching and which have possibly been eloxated to a reduced depth subsequently and additionally or which have subsequently been provided with a colloidal emulsion on the surface. Conveniently, the electrophotographic emulsion is in a thickness of from 0.001 to 0.008 mm. The procedure outlined in Example 11 is followed to produce the electrophotographic image and for the subsequent conversion into the print support.

*Example 17*

43.75 g. of triisocyanate modified in accordance with Example 12, 75% by weight in ethylacetate, and 32 g. of 2,4-di-hydroxy benzophenone are dissolved in 100 cc. of cyclohexanone and first reacted with reflux boiling at 150° C. for 10 minutes, whereafter the temperature is increased to 200° C., the cyclohexanone being distilled off. The light-yellow thickly viscous resin is dissolved hot in 90 cc. of cyclohexanone.

1 part by volume of the solution of self-adhesive photoconductor is diluted with 2 parts by volume of methyl ethyl ketone and so applied to a bright eloxated aluminium plate, to produce the photoconductive emulsion, and dried, that the emulsion thickness is 0.01 mm. The hard substantially colourless photoconductive emulsion sticks satisfactorily to the backing material and has a high storage capacity for the electric charge. If the emulsion is charged with a negative corona to 10 kv. for a short time, placed below a positive original, irradiated with ultra-violet fluorescent tubes for 10 seconds, then developed with a triboelectric developer comprising glass balls and the commercial product known as Graph-O-Fax-Toner 39/50, a high-contrast positive image of the original with high resolution is produced.

100 g. of the self-adhesive photoconductor dissolved in cyclohexanone are diluted with 50 g. of methyl ethyl ketone, 100 g. of zinc oxide (maker's name: Florence-Green No. 8) are added, and the mixture is ground in a vibrating ball mill for 2 hours. The preparation, which can readily be applied as a coating, is applied to 60 g./m.<sup>2</sup> cellulose paper to produce the photoconductive layer and is dried in a warm air stream at 120° C.

When this material is charged under a negative corona of from 6-10 kv., placed below a positive original, irradiated with ultra-violet fluorescent tubes for 0.04 second, then developed with the toner just described, a high-contrast positive image of the original is produced in which fine lines are reproduced and in which the resolution is high. The toner image can be developed by liquid developers or by toner aerosols. Fixing is effected by known steps, for instance, by heating to 120° C.

10 What I claim is:

1. An electrophotographic material comprising a carrier and an electrophotographic layer thereon, said layer containing a low molecular non-polymeric ketone of the formula



wherein

X and X<sub>1</sub> are each selected from the group consisting of halogen, —CN, —NH<sub>2</sub>, —NHR, —NR<sub>2</sub>, —OH, —OR, —SH, —SR, —COOH, —COOR, —CONH<sub>2</sub>, —CONR<sub>2</sub>, =O, =S, =SO, —SO<sub>2</sub>NH<sub>2</sub>, —SO<sub>2</sub>NHR, —SO<sub>2</sub>NR<sub>2</sub>, —NO<sub>2</sub>, —NO and aliphatic residues of 1 to 12 C-atoms;

25 and wherein

R is selected from the group consisting of an aliphatic residue of 1-12 carbon atoms, phenyl, naphthyl, diphenyl, polar substituted phenyl, naphthyl, and diphenyl,

30 wherein

the polar substituents are selected from the group consisting of —OH, —SH, —NH<sub>2</sub>, —NHCH<sub>3</sub>, —NHC<sub>2</sub>H<sub>5</sub>, —Cl, —CN or —COOH;

35 wherein

Ar and Ar<sub>1</sub> are each selected from the group consisting of mononuclear rings having aromatic properties, two mononuclear rings having aromatic properties connected to one another by a single carbon atom, and two ortho condensed mononuclear rings having aromatic properties, and wherein n is any whole number selected from 1, 2 and 3 and n<sub>1</sub> is whole numbers from zero to 3.

2. The electrophotographic material of claim 1, where 45 in the low molecular, non-polymeric ketone is reacted with an organic isocyanate, whereby the reaction products are electrophotographically active and which firmly adhere to the carrier without the addition of a separate binder, so as to form a self-adherent electrophotographic layer.

3. An electrophotographic material comprising a carrier and an electrophotographic layer thereon, said layer containing a low molecular, non-polymeric ketone of the formula



wherein

X and X<sub>1</sub> are each selected from the group consisting of halogen, —CN, —NH<sub>2</sub>, —NHR, —NR<sub>2</sub>, —OH, —OR, —SH, —SR, —COOH, —COOR, —CONH<sub>2</sub>, —CONR<sub>2</sub>, =O, =S, =SO, —SO<sub>2</sub>NH<sub>2</sub>, —SO<sub>2</sub>NHR, —SO<sub>2</sub>NR<sub>2</sub>, —NO<sub>2</sub>, —NO and aliphatic residues of 1 to 12 C-atoms;

65 and wherein

R is selected from the group consisting of an aliphatic residue of 1-12 carbon atoms, phenyl, naphthyl, diphenyl, polar substituted phenyl, naphthyl, and diphenyl,

wherein

the polar substituents are selected from the group consisting of —OH, —SH, —NH<sub>2</sub>, —NHCH<sub>3</sub>, —NHC<sub>2</sub>H<sub>5</sub>, —Cl, —CN or —COOH;

wherein

Ar and Ar<sub>1</sub> are each selected from the group consisting of mononuclear rings having aromatic properties, two mononuclear rings having aromatic properties connected to one another by a single carbon atom, and two ortho condensed mononuclear rings having aromatic properties, and wherein n is any whole number selected from the group consisting of 1, 2 and 3 and n<sub>1</sub> is any integer from zero to 3.

4. The electrophotographic material of claim 3, wherein the low molecular, non-polymeric thioketone is reacted with an organic isocyanate, whereby the reaction products are electrophotographically active and which firmly adhere to the carrier without the addition of a separate binder, so as to form a self-adherent electrophotographic layer.

5. An electrophotographic material comprising a carrier and an electrophotographic layer thereon containing a low molecular weight nonpolymeric compound selected from the group consisting of ketones and thioketones having the formula



which is reacted with an organic isocyanate compound; and wherein X and X<sub>1</sub> are each selected from the group consisting of —NHR, —NR<sub>2</sub>, —OR, —SR, —COOR, —CONHR, —CONR<sub>2</sub>, —SO<sub>2</sub>NHR, and —SO<sub>2</sub>NR<sub>2</sub>, wherein R is selected from the group consisting of -phenyl, -naphthyl, and -diphenyl, each substituted by polar constituents selected from the group consisting of —OH, —SH, —NH<sub>2</sub>, —NHCH<sub>3</sub>, —NHC<sub>2</sub>H<sub>5</sub>, —COOH, —CN, and —Cl; and wherein Y and Y<sub>1</sub> are each selected from the group consisting of —OH, —SH, —NOH and —COOH each in an ortho position of the



group; and wherein Z is selected from the group consisting of O and S.

6. An electrophotographic material comprising a carrier and an electrophotographic layer thereon containing a low molecular weight non-polymeric compound selected from the group consisting of ketones and thioketones having the formula



which is reacted with an organic epoxide compound; and wherein X and X<sub>1</sub> are each selected from the group consisting of —NHR, —NR<sub>2</sub>, —OR, —SR, —COOR, —CONHR, —CONR<sub>2</sub>, —SO<sub>2</sub>NHR, and —SO<sub>2</sub>NR<sub>2</sub>, wherein R is selected from the group consisting of -phenyl, -naphthyl, and -diphenyl, each substituted by polar constituents selected from the group consisting of —OH, —SH, —NH<sub>2</sub>, —NHCH<sub>3</sub>, —NHC<sub>2</sub>H<sub>5</sub>, —COOH, —CN, and Cl; and wherein Y and Y<sub>1</sub> are each selected from the group consisting of —OH, —SH, —NOH and —COOH each in an ortho position of the



group; and wherein Z is selected from the group consisting of O and S.

7. An electrophotographic material comprising a carrier and an electrophotographic layer thereon containing a mixture of the reaction product of claim 5 and zinc oxide.

8. An electrophotographic material comprising a carrier and an electrophotographic layer thereon containing a mixture of the reaction product of claim 6 and zinc oxide.

9. An electrophotographic material comprising a carrier and an electrophotographic layer thereon containing

a low molecular weight nonpolymeric compound selected from the group consisting of ketones and thioketones having the formula



wherein X and X<sub>1</sub> are each selected from the group consisting of -halogen, —CN, —NH-Alkyl, —N(Alkyl)<sub>2</sub>, —(Aryl)<sub>2</sub>, —OH, —O-Alkyl, —O-Aryl, —SH, —S-Alkyl, —S-Aryl, —COOH, —COO-Alkyl, —COO-Aryl, —CONH<sub>2</sub>, —CON(Alkyl)<sub>2</sub>, —COH(Aryl)<sub>2</sub>, =O, =S, =SO, —SO<sub>2</sub>NH<sub>2</sub>, —SO<sub>2</sub>NH-Alkyl, —SO<sub>2</sub>NH-Aryl, —SO<sub>2</sub>N(Alkyl)<sub>2</sub>, —SO<sub>2</sub>(Aryl)<sub>2</sub>, —NO<sub>2</sub>, -Alkyl and -Aryl; and wherein Z is selected from the group consisting of O and S; and wherein n is any whole number selected from the group consisting of 1, 2, and 3 and n<sub>1</sub> is any integer from zero to 3.

10. An electrophotographic material comprising a carrier and an electrophotographic layer thereon containing a low molecular weight nonpolymeric compound selected from the group consisting of ketones and thioketones having the formula



wherein X and X<sub>1</sub> are each selected from the group consisting of —NHR, —NR<sub>2</sub>, —OR, —SR, —COOR, —CONHR, —CONR<sub>2</sub>, —SO<sub>2</sub>NHR and —SO<sub>2</sub>NR<sub>2</sub>, and wherein R is selected from the group consisting of -phenyl, -naphthyl, and -diphenyl, each substituted by polar constituents selected from the group consisting of —OH, —SH, —NH<sub>2</sub>, —NHCH<sub>3</sub>, —NHC<sub>2</sub>H<sub>5</sub>, —COOH, —CN, and Cl, and wherein Y and Y<sub>1</sub> are each selected from the group consisting of —OH, —SH, —NOH and —COOH each in an ortho position of the

30 35 40 45 50 55 60 65 70 75 80 85 90 95

wherein Z is selected from the group consisting of O and S; and wherein n is any whole number selected from the group consisting of 1, 2 and 3 and n<sub>1</sub> is any integer from zero to 3.

11. An electrophotographic material comprising a carrier and an electrophotographic layer thereon containing a material selected from the group consisting of:

N<sup>'''</sup>,N<sup>''''</sup>-tetramethyl-di- $\alpha$ -amino-di- $\beta$ -pyridylthioketone,  
phenyl- $\alpha$ -thienyl-ketone,  
di-(quinolyl)-(6)-ketone,  
4-[methyl-( $\beta$ -hydroxyethyl)-amino]-cinnamal-4'-diphenyl-acetophenone,  
4-[methyl-( $\beta$ -hydroxyethyl)-amino]-cinnamal-3'-nitroacetophenone,  
4-dimethylamino-cinnamal-3'-amino-acetophenone,  
4-[methyl-( $\beta$ -hydroxyethyl)-amino]-cinnamal-2'-hydroxy-4'-dimethylamino-acetophenone,  
4,4'-bis(dimethylamino-dibenzylidene-acetone,  
2,2'-bis-( $\beta$ -methylamino-ethyl)-benzal,  
phenyl-(1-amino-anthraquinolyl)-(2)-ketone,  
9-hydroxy-4-benzoyl fluorene,  
 $\alpha$ -anisylidene- $\alpha$ -(3-nitro-cinnamylidene)-acetone,  
 $\alpha$ -4-[methyl-( $\beta$ -hydroxyethyl)-amino]-cinnamylidene- $\alpha$ '-(4'-nitro-toluylene)-acetone,  
4-[methyl-( $\beta$ -hydroxyethyl)-amino]-cinnamal-acetyl-acenaphthene,  
2-[2'-(carboxy-monoglycol ester)-benzoyl]-7-diethyl-amino-fluorenone,  
1,1-carbonyl-diindazole,  
1-(4'-nitrobenzoyl)-indazole,  
1-(4'-dimethylamino-benzoyl)-6-nitro-indazole,  
1-(2'-carboxyphenyl)-benzimidazole,  
2-(4''-dimethylamino-benzoyl)-3-hydroxy-diphenyl,  
2-(4''-dimethylamino-benzoyl)-3-hydroxy-4'-diethyl-aminodiphenyl,  
1-(4'-dimethyl-aminobenzoyl)-3-(4''-dimethylamino-phenyl)-indazole,  
1-(4'-diethyl-amino-benzoyl)-6-nitro-benzimidazole.

(References on following page)

## References Cited by the Examiner

## UNITED STATES PATENTS

2,710,274 6/1955 Kuehl ----- 96-89  
 3,025,160 3/1962 Bunge ----- 96-1  
 3,155,503 11/1964 Cassiers et al. ----- 96-1

## FOREIGN PATENTS

248,402 8/1960 Australia.  
 562,336 5/1958 Belgium.  
 1,249,634 11/1960 France.  
 1,060,259 6/1959 Germany.  
 1,060,713 7/1959 Germany.

1,105,713 4/1961 Germany.

## OTHER REFERENCES

Minsk et al.: J. Appl. Polym. Sci., vol. II, No. 6, 1959,  
 5 pp. 302-7.  
 Robertson et al.: J. Appl. Polym. Sci., vol. II, No. 6,  
 1959, pp. 308-311.

NORMAN G. TORCHIN, Primary Examiner.

10 A. LIBERMAN, C. E. VAN HORN,  
*Assistant Examiners.*